

(No Model.)

G. HAMMER & C. A. GREINER.  
Fire Kindler.

No. 236,889.

Patented Jan. 25, 1881.

Fig. 1.



Fig. 2.



Fig. 3.



Witnesses:

A. P. Grant,

H. F. Kirchen

Inventors:

G. Hammer,  
C. A. Greiner,  
by John A. Diederich.

ATTORNEY.

# UNITED STATES PATENT OFFICE.

GEORGE HAMMER, OF REUTLINGEN, AND CARL A. GREINER, OF NÜRTINGEN, GERMANY.

## FIRE-KINDLER.

SPECIFICATION forming part of Letters Patent No. 236,889, dated January 25, 1881.

Application filed October 30, 1880. (No model.)

*To all whom it may concern:*

Be it known that we, GEORGE HAMMER, of Reutlingen, and CARL A. GREINER, of Nürtingen, Empire of Germany, and both subjects of Germany, have invented a new and useful Improvement in Fire-Kindlers, which improvement is fully set forth in the following specification and accompanying drawings, in which—

10 Figure 1 is a top or plan view of a sheet of fire-kindlers embodying our invention. Fig. 2 is a transverse section thereof, also showing the mode of packing the kindlers. Fig. 3 is a perspective view of one of the kindlers.

15 Similar letters of reference indicate corresponding parts in the several figures.

Our invention consists of a composition of matter forming an improvement in fire-kindlers.

20 It also consists in forming the kindlers of hollow pyramidal form, whereby they may readily pack one with another and possess a large burning-surface.

It further consists of a novel striking-surface for the tips of the kindler, by which said kindler may be readily ignited, and matches are dispensed with, the tips being of such composition that they cannot be ignited without the employment of the prepared striking-surface.

25 Referring to the drawings, A represents the kindlers, which are molded of a composition of inflammable material in the form of hollow pyramids, a number of which are produced in a sheet united at their base rims, thus admitting each kindler to be easily broken off as required. The sheets may be placed one above the other, it being noticed that the apices of one sheet project into the hollow of the contiguous sheet, so that the several sheets interlock and fit each other snugly, thus providing convenient means of packing and transporting the kindlers.

30 The composition employed for the kindlers is as follows: thirty parts granulated cork, sixty parts rosin, five parts oily matter, five

parts petroleum residuum. The rosin is melted over a slow fire, the oily matter added, and cork gradually stirred in with them, after which the warm mass is poured into molds, 50 the composition readily admitting of molding, and producing a kindler which is highly inflammable, burns long without unpleasant odors, and is inexpensive.

Each kindler has its apex or point tipped 55 or dipped, as at a, with the following composition: four parts chlorate of potassium, two parts chromate of potassium, two parts vermillion or red lead, one part sulphur, one part chalk, one part sandstone, and one part gum-arabic. This provides a convenient form of 60 igniting the kindlers by friction or striking, and dispenses with matches for such purpose; but the composition is of such nature that it cannot be ignited unless when struck on a prepared surface, the latter being formed of the 65 following materials: one part amorphous phosphorus, one part grains of sulphur, and one part sulphate of antimony. This insures the safety of the kindlers, as the tips do not ignite by friction with other surfaces than one specially prepared.

Having thus described our invention, what we claim as new, and desire to secure by Letters Patent, is—

70 1. The fire-kindler composed of cork, rosin, oily matter, and petroleum residuum, substantially as and for the purpose set forth.

2. A fire-kindler of hollow pyramidal form, provided with tip a, of highly-inflammable material.

3. A sheet of hollow pyramidal fire-kindlers, connected as shown, each being provided with an inflammable tip, a, substantially as and for the purpose set forth.

4. A fire-kindler of hollow pyramidal form, substantially as and for the purpose set forth.

GEORGE HAMMER.  
C. A. GREINER.

Witnesses:

CARL OELSCHLAEGER,  
REINHOLD RIETH.